

No. 728,461.

PATENTED MAY 19, 1903

H. M. HAY.

MANIFOLD SHEET.

APPLICATION FILED NOV. 11, 1901.

NO MODEL.

FIG. 1.



FIG. 2.



Witnesses

Ric<sup>y</sup> C. Bowen.

Arthur L. Bryant.

Inventor

H. M. Hay,

By Watson Watson

Attorney

## UNITED STATES PATENT OFFICE.

HOWARD MORTON HAY, OF BROOKLYN, NEW YORK.

## MANIFOLD-SHEET.

SPECIFICATION forming part of Letters Patent No. 728,461, dated May 19, 1903.

Application filed November 11, 1901. Serial No. 81,943. (No specimens.)

*To all whom it may concern:*

Be it known that I, HOWARD MORTON HAY, a citizen of the United States, residing at Brooklyn, in the county of Kings, State of New York, have invented certain new and useful Improvements in Manifold-Sheets, of which the following is a specification.

The object of this invention is to provide a manifold-sheet adapted to produce upon the impression-sheet against which it is placed a duplicate copy in permanent copying or non-copying ink.

In the accompanying drawings, Figure 1 is a perspective view of a manifold-sheet embodying my improvements, in which *a* represents the front or printing surface of the sheet, and *b* represents the rear side of the sheet, having an impervious coating thereon; and Fig. 2 represents a cross-section through a portion of the sheet exaggerated in thickness.

Heretofore duplicate copies of manuscript or type-written matter have been made by the use of manifold-sheets consisting of thin hard paper, upon the surface of which is placed a coating consisting of soot or carbon and an adhesive material, and manifold-sheets have also been made for the purpose of obtaining more durable copies by placing upon the surface of paper sheets soluble ink or dye composition which when transferred to the impression-sheet and moistened in the act of press-copying permeates the impression-sheet and makes a permanent ink record. My manifold-sheet differs from these in that I employ instead of the hard thin paper which is ordinarily used for such purpose a thin bibulous paper thinly coated on one side with a tough flexible impervious substance, and I saturate the paper with any of the well-known non-drying inks now generally used on type-writer ribbons, whether soluble in water or not, the ink being applied in its fluid state and saturating the paper through to the impervious coating on the back. This manifold-sheet differs in its properties from those heretofore manufactured in several ways. The ink when transferred to the impression-sheet makes the same permanent copying or non-copying record which is made from a type-writer ribbon without the necessity of moistening the impression-sheet. The bibulous

paper retains a much larger quantity of ink or coloring-matter than can be retained upon the surface of the ordinary hard tissue-sheet which is generally employed, and hence will last much longer. Owing to the porous character of the paper and the fluid nature of the ink repeated use of certain portions of the paper, as when the type falls on the same parts of the paper repeatedly, will not exhaust the coloring-matter from such parts nor cause them to print distinctly fainter than the unused parts after the manifold-paper has been used a few times, for the reason that the ink is constantly drawn by capillary attraction to the points from whence ink has been transferred by the impression of the type to the impression-sheets. The flexible impervious coating while providing a clean side to the sheet holds the fibers of the latter together at the back of the sheet and returns them to their normal position after the impression of the type, and thus prevents the destruction of the sheet.

In preparing my new manifold-sheet I take a thin bibulous paper similar to ordinary blotting-paper, but much thinner, and I coat it upon one side with a thin coating of collodion, which dries almost as quickly as it can be applied. A non-drying ink, either copying or non-copying, such as is commonly used on type-writer ribbons, is then applied in its fluid state to the opposite side of the sheet, the latter becoming thoroughly saturated therewith. The collodion coating on the back of the sheet is impervious to the ink and is sufficiently tough and flexible to yield without breaking under the impression of the type and by its adhesion to the fibers of the paper returns the latter to their normal condition. The surplus ink, if any, is removed from the surface of the manifold-sheet by pressing any suitable absorbent sheet against it, and the manifold-sheet is then preferably exposed to the atmosphere for a sufficient length of time before using to permit the ink to become evenly distributed throughout the fibers by capillary attraction and the outer surface to become dry enough to be handled without smearing.

Having thus fully described my invention, what I claim, and desire to secure by Letters Patent, is—

1. As a new article of manufacture, a mani-

fold-sheet consisting of a thin bibulous paper having a coating on one side impervious to ink and saturated through to said coating with a non-drying ink.

- 5 2. As a new article of manufacture, a mani-fold-sheet consisting of a thin bibulous paper having a flexible coating on one side impervious to ink and saturated through to said coating with a non-drying ink.
- 10 3. As a new article of manufacture, a mani-

fold-sheet consisting of a thin bibulous paper having a coating of collodion on one side and saturated through to said coating with a non-drying ink.

In testimony whereof I affix my signature 15 in presence of two witnesses.

HOWARD MORTON HAY.

Witnesses:

HENRY JOSEPH NOLLER,  
ARTHUR WARD OAKLEY.